

# UNITED STATES PATENT OFFICE.

DEWITT T. BECKHAM, OF GENEVA, TEXAS.

## PROCESS FOR HARDENING COPPER.

1,331,479.

Specification of Letters Patent.

Patented Feb. 24, 1920.

No Drawing.

Application filed March 13, 1919. Serial No. 282,373.

*To all whom it may concern:*

Be it known that I, DEWITT T. BECKHAM, a citizen of the United States, residing at Geneva, in the county of Sabine and State 5 of Texas, have invented certain new and useful Improvements in Processes for Hardening Copper, of which the following is a specification.

This invention relates to improvements in metal and it is the principal object of the invention to provide a novel and simple process for hardening copper embracing steps whereby a bending or scaling of a body of such metal subsequent to the hardening of the same by the improved process will be positively prevented.

In order that the invention may be readily understood by those skilled in the art, I have in the detailed following description 20 based thereon set forth a preferred embodiment of the invention.

To harden copper in accordance with my novel process, I first heat the same to a certain temperature, either to red glow at 25 a temperature of 1370 degrees Fahrenheit or to incandescence at a temperature of 1950 degrees Fahrenheit. Immediately subsequent to the heating of the metal to the desired temperature it is subjected to material 30 pressure, such as by hammering or like operations until the metal body is cold. The hammering of the metal body will serve to close the pores thereof, thus rendering the same exceedingly hard. Due to the heating 35 of the metal before the hammering of the same, I desire to have it understood that the scaling thereof will be eliminated, that is the appearance of flakes on the hammered surfaces of the metal will be prevented. As

will be understood, some difficulty has heretofore been experienced when methods or processes for hardening copper have been introduced embracing the hammering of metal as one of the steps thereof. However, by heating the metal previous to the hammering of the same for tempering and for opening the pores of the body, I entirely overcome this difficulty.

I have found from actual experiments that the heating of the metal in addition to causing expansion and the resultant opening of the pores of a metal body will also impart a certain amount of pliability to the same and in consequence successfully withstand the impacts thereon by reason of the hammering and prevent scaling or flaking. I have also ascertained through actual experiments that by heating the metal body to be hardened to a red glow and then hammering it, it will become sufficiently hard for various purposes. However, by heating the metal body to an incandescence and then hammering the same, the metal becomes very hard and brittle and cannot be bent without fracturing the same.

I claim:

1. The herein described process of hardening copper consisting of heating the same to a high temperature and then hammering it until cold.

2. The herein described process of hardening copper consisting of heating the same to a high temperature and then subjecting it to continual pressure until cold.

In testimony whereof, I affix my signature hereto.

DEWITT T. BECKHAM.